

Patented Dec. 16, 1952

2,621,789

## UNITED STATES PATENT OFFICE

2,621,789

FROTH FLOTATION OF SULFIDE MINERALS  
WITH DI-ALKYL THIOPHOSPHORYL  
CHLORIDES

Robert B. Booth, Stamford, and Charles L. Morris,  
Jr., Noroton Heights, Conn., assignors to Ameri-  
can Cyanamid Company, New York, N. Y., a  
corporation of Maine

No Drawing. Application October 4, 1950,  
Serial No. 188,478

14 Claims. (Cl. 209—166)

1

This invention relates to an improved method of froth flotation of sulfide ores using a new type of reagent.

The standard methods of floating sulfide ores involve the use of two principal types of reagent. The first are the various xanthates; and the second, esters of dithiophosphoric acid. While these reagents are extremely effective in most sulfide flotation and account for the large bulk of sulfides recovered by froth flotation, they are less effective especially in certain circuits, i. e. those which are strongly acid. For this special type of froth flotation, there have been developed special promoters or collectors in which xanthates are condensed with various other compounds. Among the most commonly used constitute reaction products of various chloroformates with xanthates of which ethyl xanthogen ethyl formate is one of the most efficient. While the special condensed xanthate reagents have enjoyed marked success in special acid circuit flotations, they still leave something to be desired in recovery.

The present invention utilizes a new type of flotation promoter or collector, namely dialkyl thiophosphoryl chlorides. This is an unusual type of reagent because generally promoters are used in the form of free acids or salts. The reactivity of acid chlorides is normally so great that such compounds could not be considered practical for froth flotation because of instability. It is not known why the dialkyl thiophosphoryl chlorides of the present invention are so stable, particularly in the acid circuits in which they are used and it is not desired to limit the present invention to any theory of why these acid chlorides should exhibit such an abnormal stability. The reagents of the present invention may be represented by the following type formula:



in which R and R' are alkyl radicals.

When the reagents of the present invention are used, substantial increases in recovery are obtained over former reagents and in some favorable circumstances giving recoveries approaching quantitative.

The efficiency will vary somewhat with different members of the series. In general, however, they appear to give improved results over the standard reagents hitherto used. Sulfide flotations which give high recoveries, even with standard reagents, present an important economic problem because many of the ores, such as copper ores, have only one to two percent of copper and increases in recovery make very substantial cost savings.

2

It is an advantage of the present invention that any of the ordinary alkyl groups may be present in the promoter. The cheapest alkyl thiophosphoryl chlorides are those in which the alkyl groups are the same, and as these compounds are just as efficient as those in which the alkyl groups are different, they are preferred. However, the invention is not limited thereto and mixed compounds may be used where R is an alkyl group and R' is a different one. Typical of such compounds are methyl, ethyl, ethyl isopropyl, etc.

Many of the alkyl thiophosphoryl chlorides are obtainable in relatively pure form. It is not, however, necessary to use highly purified compounds and crude products give reasonably satisfactory results and, in some cases, represent an economical advantage.

The invention will be described in greater detail in conjunction with the following specific examples. It is to be understood that these examples are set forth for the purpose of illustration only and are not to be considered as limitations on the case, except as indicated by the appended claims.

## Example 1

A South American copper ore (about 1.9–2.0% Cu) was ground in separate tests with various dialkyl thiophosphoryl chlorides to minus 65 mesh and then conditioned with 8.0 16/ton sulfuric acid and 0.24 16/ton cresylic acid. The resulting pulp was floated in a Fagergren flotation machine at 22% solids for 7.5 minutes. A comparative test was carried out with ethyl xanthogen ethyl formate added to the grind; this material is the standard promoter for this ore. The following metallurgical results were obtained:

| 40 | Promoter Used                                                 | Concentrate |            |        | Tailing-Percent Cu Assay |  |
|----|---------------------------------------------------------------|-------------|------------|--------|--------------------------|--|
|    |                                                               | Percent Wt. | Percent Cu |        |                          |  |
|    |                                                               |             | Assay      | Recov. |                          |  |
| 45 | 0.3 16/ton Ethyl xanthogen ethyl formate                      | 13.6        | 12.80      | 80.4   | 0.49                     |  |
|    | 0.3 16/ton Dimethyl thiophosphoryl chloride                   | 13.3        | 12.62      | 85.4   | 0.33                     |  |
|    | 0.3 16/ton Diethyl thiophosphoryl chloride                    | 13.7        | 12.01      | 86.0   | 0.31                     |  |
| 50 | 0.3 16/ton Di-sec. butyl thiophosphoryl chloride <sup>1</sup> | 15.6        | 10.31      | 85.6   | 0.32                     |  |

<sup>1</sup> Crude products.

## Example 2

A copper-bearing slime from the northwestern part of the United States (90% minus 325 mesh; about 1.6–1.7% Cu in copper content) was con-

ditioned with 0.2 16/ton of diethyl thiophosphoryl chloride and 0.13 16/ton pine oil and floated in a Fagergren flotation machine for 6 minutes. A concentrate, assaying 7.01% Cu and containing 84.3% of the total copper was obtained; the tailings assayed 0.14% Cu.

A corresponding test with 0.2 16/ton of ethyl xanthogen ethyl formate recovered 80.0% of the copper in a concentrate assaying 6.25% Cu; the tailing assayed 0.26% Cu.

*Example 3*

Diethyl thiophosphoryl chloride and diisopropyl thiophosphoryl chloride were used also as promoters on a zinc ore from the southeastern part of the United States. This ore was ground to about 65 mesh and conditioned with 0.075 lb./ton of each promoter and 0.065 lb./ton pine oil as frother. The resulting pulp was floated in a Fagergren flotation machine for 5 minutes. The metallurgical results were as follows:

| Promoter Used                       | Concentrate        |             |        | Tailing--<br>Per Cent<br>Zn Assay |  |
|-------------------------------------|--------------------|-------------|--------|-----------------------------------|--|
|                                     | Per<br>Cent<br>Wt. | Per Cent Zn |        |                                   |  |
|                                     |                    | Assay       | Recov. |                                   |  |
| Diethyl thiophosphoryl chloride     | 2.64               | 43.99       | 97.51  | 0.07                              |  |
| Diisopropyl thiophosphoryl chloride | 2.61               | 47.00       | 96.74  | 0.09                              |  |

**We claim:**

1. A method of beneficiating sulfide ores by froth flotation which comprises effecting the froth flotation in the presence of a promoter having the following formula:



in which R and R' are alkyl groups, recovering a froth concentrate relatively rich in the sulfide mineral and obtaining a froth tailing relatively poor in the sulfide mineral.

2. A method according to claim 1 in which the sulfide ore is a copper sulfide ore.

3. A method according to claim 2 in which the promoter is dimethyl thiophosphoryl chloride.

4. A method according to claim 1 in which the ore is a copper sulfide ore and the promoter is diethyl thiophosphoryl chloride.

5. A method according to claim 1 in which the ore is a copper sulfide ore and the promoter is diisopropyl thiophosphoryl chloride.

6. A method according to claim 1 in which the ore is a copper sulfide ore and the promoter is di-sec. butyl thiophosphoryl chloride.

7. A method according to claim 1 in which the ore is a zinc sulfide ore.

8. A method according to claim 7 in which the promoter is diethyl thiophosphoryl chloride.

9. A method according to claim 1 in which flotation is effected in acid circuit.

10. A method according to claim 9 in which the sulfide ore is a copper sulfide ore.

11. A method according to claim 10 in which the promoter is dimethyl thiophosphoryl chloride.

12. A method according to claim 9 in which the flotation is effected in acid circuit, the ore is a copper sulfide ore and the promoter is diethyl thiophosphoryl chloride.

13. A method according to claim 9 in which the flotation is effected in acid circuit, the ore is a copper sulfide ore and the promoter is diisopropyl thiophosphoryl chloride.

14. A method according to claim 9 in which the flotation is effected in acid circuit, the ore is a copper sulfide ore and the promoter is di-sec. butyl thiophosphoryl chloride.

ROBERT E. BOOTH.  
CHARLES L. MORRIS, JR.

**REFERENCES CITED**

40 The following references are of record in the file of this patent:

**UNITED STATES PATENTS**

| Number       | Name           | Date           |
|--------------|----------------|----------------|
| 45 1,812,839 | Derby          | June 30, 1931  |
| 1,893,018    | Christmann     | Jan. 3, 1933   |
| 2,482,063    | Hechenbleikner | Sept. 13, 1949 |